

## 1

3,532,639

**CORROSION INHIBITING WITH COMBINATIONS OF ZINC SALTS, AND DERIVATIVES OF METHANOL PHOSPHONIC ACID**

 George B. Hatch, Allison Park, Pa., assignor to  
 Calgon Corporation, Pittsburgh, Pa.

 No Drawing. Filed Mar. 4, 1968, Ser. No. 709,951  
 Int. Cl. C23f 11/10, 11/16

U.S. Cl. 252—389

10 Claims

**ABSTRACT OF THE DISCLOSURE**

Novel combinations of zinc salts and derivatives of methanol phosphonic acid or methanol diphosphonic acid are used in small concentrations to inhibit corrosion in aqueous systems.

**BACKGROUND OF THE INVENTION**

This invention relates to corrosion inhibitors for aqueous systems. In the past, the corrosion inhibitors in most widespread use have contained either inorganic polyphosphates or chromates, while the polyphosphates have a tendency to hydrolyze and revert to orthophosphates, the waste disposal problems posed by toxic chromate containing corrosion inhibitors have resulted in increased demand for corrosion inhibitors of a completely different class.

Certain derivatives of methanol phosphonic acids have been disclosed in the literature. Alkyl and aryl alpha hydroxyphosphonic acids and salts thereof long have been known. See for example, Monatsch 5, 120,627 (1884); J. Am. Chem. Soc. 42, 2337 (1920); J. Am. Chem. Soc. 43, 1928 (1921); Belgian Pat. 678,912. See also U.S. Pat. 3,122,417 and U.S. Pat. 3,214,454. U.S. Pat. 3,159,581 shows the use of such compounds in detergent compositions. Also of interest are Belgian Pats. 655,166 and 672,168. In U.S. Pat. 3,122,417, mentioned above, a series of alkyl alpha-hydroxy 1,1-diphosphonic acid is disclosed. The distinctive common feature of the compounds of present interest is the presence of one or more alpha-hydroxy phosphonic acid groups. These groups may be represented by the following formula:



where R is H, a lower alkyl group or



TABLE II.—INHIBITION OF CORROSION OF STEEL BY COMBINATIONS OF ZINC SULFATE WITH COMPOUNDS CONTAINING METHANOL DIPHOSPHONATE GROUPS (pH 6.8-7)

| Phosphonate conc. (p.p.m.) | Zinc (sulfate) conc. (p.p.m. Zn) | Weight loss (m.d.d.)        |                                      |                                    |      |
|----------------------------|----------------------------------|-----------------------------|--------------------------------------|------------------------------------|------|
|                            |                                  | Sodium methanol phosphonate | Sodium dimethyl methanol phosphonate | Sodium phenyl methanol phosphonate |      |
| 0                          | 0                                | 0                           | 187                                  | 108                                | 43.1 |
| 10                         | 3                                | 107                         | 108                                  | 5.2                                |      |
| 15                         | 4.5                              | 51.4                        | 9.6                                  | 3.5                                |      |
| 20                         | 6                                | 25.4                        | 5.5                                  | 3.8                                |      |
| 30                         | 9                                | 4.0                         | 2.2                                  | 3.9                                |      |
| 50                         | 15                               | 4.6                         |                                      |                                    |      |

Table II shows the effectiveness of combinations of zinc sulfate with compounds containing methanol diphosphonate groups. The quantities of zinc supplied were equal to 30% of the methanol diphosphonate concentrations.

TABLE II.—INHIBITION OF CORROSION OF STEEL BY COMBINATIONS OF ZINC SULFATE WITH COMPOUNDS CONTAINING METHANOL DIPHOSPHONATE GROUPS (pH 6.8-7)

| Phosphonate conc. (p.p.m.) | Zinc (sulfate) conc. (p.p.m. Zn) | Methyl methanol diphosphonate | Sodium phenyl methanol diphosphonate | Sodium methylene bis (methanol diphosphonate) | Sodium dimethylene bis (methanol diphosphonate) | Sodium tetramethylene bis (methanol diphosphonate) |
|----------------------------|----------------------------------|-------------------------------|--------------------------------------|-----------------------------------------------|-------------------------------------------------|----------------------------------------------------|
| 0                          | 0                                | 77.8                          | 82.9                                 | 118                                           | -----                                           | -----                                              |
| 5                          | 1.5                              | 2.0                           | 19.9                                 | 1.0                                           | 9.8                                             | 75.2                                               |
| 10                         | 3                                | 2.3                           | 4.4                                  | 1.2                                           | 4.6                                             | 23.3                                               |
| 15                         | 4.5                              | 1.8                           | 2.2                                  | 1.0                                           | 0.7                                             | 0.6                                                |
| 20                         | 6                                | 1.6                           | 2.6                                  | 2.4                                           | 2.4                                             | 0.6                                                |
| 30                         | 9                                | 2.8                           | 2.6                                  | 0.9                                           | 1.1                                             | 0.7                                                |
| 50                         | 15                               |                               |                                      |                                               |                                                 |                                                    |

They may be considered as methanol phosphonic acid or where R is



as methanol diphosphonic acid groups.

 2  
**SUMMARY OF THE INVENTION**

I have discovered that combinations of zinc salts with compounds containing one or more methanol phosphonic or methanol diphosphonic groups or soluble salts thereof provide excellent inhibition of corrosion of metals, particularly iron and steel, in aqueous systems.

Some particular compounds which are useful in my invention may be represented by the formula



where  $R_1$  is independently selected from the group consisting of H, alkyl groups up to four carbon atoms, phenyl, and phosphonate groups,  $R_2$  is hydrogen, an alkyl group having up to four carbon atoms or



where  $n$  is 0 to 8, and water soluble salts thereof.

The effectiveness of combinations of zinc sulfate with the sodium salts of the methanol phosphonic acids is shown in Table I. The zinc sulfate additions were calculated to supply zinc in amounts equal to 30% of the sodium methanol phosphonate concentrations. These examples as well as all the examples in this disclosure, were obtained by immersing steel samples in the solutions described under agitation for five days at 35°C. The pH in Table I was 6.8. Weight loss results are stated in terms of milligrams per square decimeter per day.

TABLE I.—INHIBITION OF CORROSION OF STEEL BY COMBINATIONS OF ZINC SULFATE WITH COMPOUNDS CONTAINING METHANOL PHOSPHONATE GROUPS (pH 6.8-7)

| Phosphonate conc. (p.p.m.) | Zinc (sulfate) conc. (p.p.m. Zn) | Weight loss (m.d.d.)        |                                      |                                    |      |
|----------------------------|----------------------------------|-----------------------------|--------------------------------------|------------------------------------|------|
|                            |                                  | Sodium methanol phosphonate | Sodium dimethyl methanol phosphonate | Sodium phenyl methanol phosphonate |      |
| 0                          | 0                                | 0                           | 187                                  | 108                                | 43.1 |
| 10                         | 3                                | 107                         | 108                                  | 5.2                                |      |
| 15                         | 4.5                              | 51.4                        | 9.6                                  | 3.5                                |      |
| 20                         | 6                                | 25.4                        | 5.5                                  | 3.8                                |      |
| 30                         | 9                                | 4.0                         | 2.2                                  | 3.9                                |      |
| 50                         | 15                               | 4.6                         |                                      |                                    |      |

Table II shows the effectiveness of combinations of zinc sulfate with compounds containing methanol diphosphonate groups. The quantities of zinc supplied were equal to 30% of the methanol diphosphonate concentrations.

TABLE II.—INHIBITION OF CORROSION OF STEEL BY COMBINATIONS OF ZINC SULFATE WITH COMPOUNDS CONTAINING METHANOL DIPHOSPHONATE GROUPS (pH 6.8-7)

| Phosphonate conc. (p.p.m.) | Zinc (sulfate) conc. (p.p.m. Zn) | Methyl methanol diphosphonate | Sodium phenyl methanol diphosphonate | Sodium methylene bis (methanol diphosphonate) | Sodium dimethylene bis (methanol diphosphonate) | Sodium tetramethylene bis (methanol diphosphonate) |
|----------------------------|----------------------------------|-------------------------------|--------------------------------------|-----------------------------------------------|-------------------------------------------------|----------------------------------------------------|
| 0                          | 0                                | 77.8                          | 82.9                                 | 118                                           | -----                                           | -----                                              |
| 5                          | 1.5                              | 2.0                           | 19.9                                 | 1.0                                           | 9.8                                             | 75.2                                               |
| 10                         | 3                                | 2.3                           | 4.4                                  | 1.2                                           | 4.6                                             | 23.3                                               |
| 15                         | 4.5                              | 1.8                           | 2.2                                  | 1.0                                           | 0.7                                             | 0.6                                                |
| 20                         | 6                                | 1.6                           | 2.6                                  | 2.4                                           | 2.4                                             | 0.6                                                |
| 30                         | 9                                | 2.8                           | 2.6                                  | 0.9                                           | 1.1                                             | 0.7                                                |
| 50                         | 15                               |                               |                                      |                                               |                                                 |                                                    |

The influence of the zinc in combination with ethanol 1,1'-diphosphonic acid is shown in Table III. Zinc in amounts equal to 30% of the ethanol 1,1'-diphosphonic acid (EDP) was added as the sulfate. Inclusion of zinc markedly improves the inhibitive action of the ethanol 1,1'-diphosphonic acid.

TABLE III.—INHIBITION OF CORROSION OF STEEL WITH ETHANOL 1,1-DIPHOSPHONIC ACID (EDP) AND INFLUENCE THEREON ON ZINC

| EDP concentration (p.p.m.) | Weight loss (m.d.d.) |                     |
|----------------------------|----------------------|---------------------|
|                            | Alone                | With zinc (30% EDP) |
| 0                          | 187                  | 77.8                |
| 5                          | 122                  | 2.0                 |
| 10                         | 95.4                 | 1.8                 |
| 20                         | 53.8                 | 1.6                 |
| 30                         | 10.2                 | 2.8                 |
| 50                         | 12.5                 | 1.8                 |
| 100                        |                      |                     |

Zinc salts produce a similar pronounced improvement of the inhibitive action of the other methanol phosphonate and diphosphonates. For example, Table IV shows the influence of zinc sulfate on inhibition of the corrosion of steel with sodium methylene bis(methanol diphosphonate) at pH 6.8-7.

TABLE IV.—INHIBITION OF CORROSION OF STEEL WITH SODIUM METHYLENE BIS(METHANOL DIPHOSPHONATE) AND INFLUENCE THEREON OF ZINC [pH=6.8-7]

| Diphosphonate conc. (p.p.m.) | Weight loss (m.d.d.) |                                  |
|------------------------------|----------------------|----------------------------------|
|                              | Alone                | With zinc (30% of diphosphonate) |
| 0                            | 187                  | 118                              |
| 5                            | 102                  | 1.0                              |
| 10                           | 72.5                 | 1.0                              |
| 20                           | 23.9                 | 2.4                              |
| 30                           | 12.7                 | 0.9                              |
| 50                           | 7.6                  |                                  |
| 100                          |                      |                                  |

The influence of the ratio of zinc to ethanol 1,1'-diphosphonic acid is shown in Table V. The ethanol 1,1'-diphosphonic acid level in these tests was constant (10 p.p.m.). The inhibition increases as the zinc level is raised to about 30% (by weight) of the ethanol 1,1'-diphosphonic acid concentration, but subsequent increases produce no further improvement.

TABLE V

Influence of zinc ( $ZnSO_4$ ) on inhibition of corrosion of steel at a fixed ethanol 1,1'-diphosphonic acid level (10 p.p.m.) pH=6.8-7

| Zn conc. (percent of EDA conc.): | Weight loss (m.d.d.) |
|----------------------------------|----------------------|
| 0                                | 118                  |
| 5                                | 112                  |
| 10                               | 45.6                 |
| 20                               | 29.4                 |
| 30                               | 2.1                  |
| 40                               | 2.1                  |
| 50                               | 2.2                  |

The combination of zinc with the substituted methanol phosphonic or diphosphonic acid compounds provides very effective inhibition of the corrosion of iron and steel over a rather wide range of pH as is illustrated by the data for the zinc-ethanol 1,1'-diphosphonic acid combination in Table IV. Inhibition starts to fall off as the pH is lowered to 5 so that appreciably lower pH levels are undesirable. Inhibition tends to fall off somewhat when the pH is raised much above 9, although it remains appreciable at pH 10.4 or above.

The methanol phosphonic and diphosphonic acid compounds are corrosive to copper and copper alloys. The presence of zinc markedly inhibits the corrosive action of these methanol phosphonic and diphosphonic acids with regards to copper and its alloys.

TABLE VI.—INHIBITOR OF CORROSION OF STEEL AT SEVERAL pH LEVELS WITH ETHANOL 1,1'-DIPHOSPHONIC ACID AND ZINC (SULFATE)

| EDP conc. (p.p.m.) | Zn <sup>2+</sup> conc. (p.p.m.) | Weight loss (m.d.d.) |          |          |            |          |
|--------------------|---------------------------------|----------------------|----------|----------|------------|----------|
|                    |                                 | pH 4.9-5.1           | pH 6-6.2 | pH 6.8-7 | pH 7.9-8.1 | pH 9-9.2 |
| 0                  | 0                               | 183                  | 181      | 187      | 152        | 110      |
| 10                 | 3                               | 16.4                 | 2.8      | 2.0      | 1.4        | 3.4      |
| 15                 | 4.5                             | 5.5                  | 2.6      | 2.3      | 3.1        | 3.2      |
| 20                 | 6                               | 6.6                  | 2.8      | 1.8      | 2.8        | 3.2      |
| 25                 | 7.5                             | 6.9                  | 4.0      | 1.8      | 2.3        | 3.4      |

Table VII shows the effect of 50 p.p.m. ethanol 1,1'-diphosphonic acid on the corrosion of copper at several pH levels and the influence thereon of 15 p.p.m. of zinc (added as the sulfate). The ethanol 1,1'-diphosphonic acid accelerates the attack throughout the pH range of 4 to 9. 15 p.p.m. zinc (30% of the EDA concentration) counteracts this accelerative action of the ethanol 1,1'-diphosphonic acid at a pH of 6, while at higher pH levels the mixture becomes inhibitive with respect to copper.

TABLE VII.—INFLUENCE OF pH ON CORROSION OF COPPER AND EFFECT THEREON OF ETHANOL 1,1'-DIPHOSPHONIC ACID (50 p.p.m.) AND MIXTURE THEREOF WITH ZINC (15 p.p.m.)

| pH | Weight loss (m.d.d.) |               |                                           |
|----|----------------------|---------------|-------------------------------------------|
|    | Untreated            | 50 p.p.m. EDP | 50 p.p.m. EDP, 15 p.p.m. Zn <sup>2+</sup> |
| 4  | 4.8                  | 12.1          | 12.5                                      |
| 5  | 2.6                  | —             | 6.5                                       |
| 6  | 2.0                  | 9.6           | 1.9                                       |
| 7  | 1.6                  | 6.9           | 0.5                                       |
| 8  | 1.3                  | 3.2           | 0.4                                       |
| 9  | 0.9                  | 3.2           | 0.1                                       |

Where lower pH values are involved or where even greater inhibition of corrosion of copper and copper alloys is desired, we have found that this may be accomplished by incorporation of the specific copper inhibitors described by Hatch in U.S. Pats. 2,941,953 and 2,742,369 with the methanol phosphonates or diphosphonates and zinc. These specific copper inhibitors include 1,2,3 triazoles (U.S. Pat. 2,941,953) (e.g. benzotriazole) and the thiols of thiazoles (e.g. 2-mercaptopbenzothiazole), oxazoles (e.g. 2-mercaptopbenzoxazole) or imidazoles (e.g. 2-mercaptopbenzimidazole) (U.S. Pat. 2,742,369).

Concentration levels of 0.05 to 5 p.p.m., preferably 0.5 to 2 p.p.m., of these triazoles or thiols should be employed when they are used in conjunction with the methanol phosphonate or diphosphonate and zinc inhibitors.

I may use any inorganic zinc salts capable of forming zinc ions in solution, i.e. water-soluble salts. Examples of such zinc salts are zinc chloride, zinc acetate, zinc nitrate, and zinc sulfate. I prefer to use zinc sulfate because it is readily available, economical and not excessively hydroscopic.

The ratio of zinc to organic phosphonate compound may vary from about 1:10 to about 1:2, by weight. Preferably the zinc will be about 20% to 40% of the weight of the organic phosphonate. Where triazoles or thiazoles as described above are used, they may be present in the inhibitor composition in amounts up to 10% by weight, preferably between 1 and 5%. Within the limits of these ranges, the concentrations of my inhibitor combination may vary from about 5 p.p.m. to 0.2% or more. At least about 5 p.p.m. of the inhibitor combination should be present in the aqueous system. Concentrations above 100 p.p.m. generally do not significantly improve the inhibition rate in cooling water and are unnecessary.

My inhibitor compositions are useful in such aqueous solution systems as cooling waters, heating systems, and certain process and distribution systems.

I do not intend to be restricted to the above illustrated specific examples. My invention may be otherwise practiced within the scope of the following claims.

I claim:

1. Composition useful for inhibiting corrosion in aqueous systems, consisting essentially of one part by weight zinc in the form of a water soluble zinc salt and from 1 to 10 parts by weight of a water-soluble organic phosphonate compound having the formula



where  $\text{R}_1$  is independently selected from the group consisting of H, alkyl groups up to four carbon atoms, phenyl, and phosphonate groups, and  $\text{R}_2$  is selected from the group consisting of hydrogen, alkyl groups having up to 4 carbon atoms and



where  $n$  is 0 to 8, and water-soluble salts thereof.

2. Composition of claim 1 in which the water-soluble zinc salt is zinc sulfate.

3. Composition of claim 1 in which the methanol phosphonate derivative is ethanol 1,1'-diphosphonic acid or water-soluble salt thereof.

4. Composition of claim 1 in which the weight ratio of zinc to the methanol phosphonate derivative is about 1 to 10 to about 1 to 2.

5. Method of inhibiting corrosion in aqueous systems comprising adding to said aqueous system at least about 5 parts per million of the composition of claim 1.

6. Method of inhibiting corrosion in aqueous systems comprising adding to said aqueous system at least about 5 parts per million of the composition of claim 2.

7. Method of inhibiting corrosion in aqueous systems comprising adding to said aqueous system at least about 5 parts per million of the composition of claim 3.

8. Method of inhibiting corrosion in aqueous systems comprising adding to said aqueous system at least about 5 parts per million of the composition of claim 4.

9. Composition of claim 1 including a copper corrosion inhibitor selected from the group consisting of 1, 2, 3 triazoles, thiols of thiazoles, oxazoles, and imidazoles, said copper corrosion inhibitor being present in an amount up to about 10% by weight.

10. Method of inhibiting corrosion in aqueous systems comprising maintaining therein an amount of the composition of claim 9 to provide up to about 5 p.p.m. copper corrosion inhibitor.

#### References Cited

#### UNITED STATES PATENTS

3,483,133 12/1969 Hatch et al. \_\_\_\_\_ 252—389

LEON D. ROSDOL, Primary Examiner

I. GLUCK, Assistant Examiner

U.S. Cl. X.R.

21—2.7; 252—8.55, 387; 260—502.4; 106—14

**Disclaimer**

3,532,639.—*George B. Hatch*, Allison Park, Pa. CORROSION INHIBITING WITH COMBINATIONS OF ZINC SALTS, AND DERIVATIVES OF METHANOL PHOSPHONIC ACID. Patent dated Oct. 6, 1970. Disclaimer filed Aug. 10, 1972, by the inventor, the assignee, *Calgon Corporation*, assenting.

Hereby enters this disclaimer to claims 1 through 10 of said patent.

[*Official Gazette February 19, 1974.*]